

1

3,210,277  
STABILISATION OF CHLORINATED  
HYDROCARBONS

George Edward Swift, Buncorn, England, assignor to Imperial Chemical Industries Limited, London, England, a corporation of Great Britain

No Drawing. Filed Aug. 10, 1964, Ser. No. 388,720  
Claims priority, application Great Britain, Aug. 26, 1963,  
33,698/63

10 Claims. (Cl. 252—42.7)

The present invention relates to the stabilisation of chlorinated hydrocarbons. More particularly it relates to the stabilisation of liquid chlorinated long chain paraffinic hydrocarbons for use as oil additives.

It is known to improve the properties of mineral oil lubricants when working under heavy loads by incorporating therein a proportion of relatively involatile liquid chlorinated paraffinic hydrocarbon, for instance a paraffinic hydrocarbon containing at least eight carbon atoms per molecule and chlorinated to a chlorine content of at least 25% by weight, particularly 40–70% by weight. Although the extreme pressure lubricant properties of mineral oils are considerably improved by such additions, the improved lubricants are found to have the disadvantage of staining metal surfaces with which they come into contact in use, as for instance in metal cutting and drawing operations and in lubricated gear assemblies.

We have now found that the aforementioned disadvantage can be avoided by incorporating in chlorinated paraffins that are to be employed as oil additives a stabiliser system comprising a barium, calcium or magnesium alkyl phenate and a sequestering agent.

According to the present invention a stabilised lubricating oil additive comprises at least one liquid chlorinated paraffinic hydrocarbon containing 8–26 carbon atoms per molecule and at least 25% by weight of chlorine, 0.1–5% of a barium, calcium or magnesium alkyl phenate as hereinafter defined and 0.1–5% of an oil-soluble sequestering agent for heavy metals, the percentages of the said phenate and the said sequestering agent being calculated on the weight of chlorinated paraffinic hydrocarbon.

The barium, calcium and magnesium phenates employed in the present invention have in their simplest form the structure:



where M is an atom of barium, calcium or magnesium, R<sub>1</sub> is hydrogen or an alkyl group containing 1–10 carbon atoms, and R<sub>2</sub> is an alkyl group containing 1–10 carbon atoms. When R<sub>1</sub> as well as R<sub>2</sub> is an alkyl group R<sub>1</sub> will usually be the same as R<sub>2</sub> since such compounds are the more easily prepared. The phenate employed may, however, contain additionally a proportion of sulphur in the form of a single sulphur linkage or a dithio linkage between the two aromatic nuclei. The formulae of such phenates may be represented by the following two structures I and II, such compounds being alternatively known as alkyl phenol sulphides and disulphides:



2

Furthermore the phenates employed may be those known to be obtained by neutralising a parent phenol with an excess of barium, calcium or magnesium hydroxide, i.e. they may be over-based so that they contain a proportion of free hydroxyl groups, for instance compounds of type I above may contain a proportion of material represented by the formula:



10 where M, R<sub>1</sub> and R<sub>2</sub> are as defined in the preceding paragraph.

Suitable sequestering agents are for instance the pentaerythritol esters of long chain fatty acids, such as oleic, stearic and lauric acids, and the alkyl and aryl phosphites.

20 The alkyl phenate and the sequestering agent may each usefully be employed to the extent of 5% by weight of the chlorinated paraffinic hydrocarbon, although for most applications 0.1–1% by weight will be found to give adequate protection against metal staining. Greater amounts than 5% by weight may be employed but such amounts give no technical advantage and in general they are not economic.

25 As stated hereinbefore, chlorinated paraffinic hydrocarbons containing 8–26 carbon atoms per molecule and at least 25% by weight of chlorine may be employed in the stabilised lubricating oil additives of the invention. Of this range of compounds we prefer to employ for most applications those containing 40–70% by weight of chlorine.

30 It is already known to add stabilisers to chlorinated hydrocarbons of the aforesaid range for the purpose of inhibiting decomposition by heat. It must be understood that chlorinated hydrocarbons stabilised according to the present invention may additionally contain conventional heat stabilisers, for example epoxidised oils.

35 We have found that if 0.1–5% by weight of a barium, calcium or magnesium alkyl phenate is added to the chlorinated hydrocarbon without an accompanying sequestering agent the staining of metal surfaces is prevented but that the heat stability of the chlorinated hydrocarbon (as determined by the standard test of measuring hydrogen chloride evolution on blowing nitrogen through the material heated for 4 hours at 175° C.) is thereby reduced, even when conventional heat stabilisers such as epoxidised oils are present. We have found, however, that addition of an oil-soluble sequestering agent for heavy metals prevents this deleterious effect, possibly by inactivating barium, calcium and magnesium chlorides which are thought to be formed in traces in the respective mixtures and to have a catalytic effect on decomposition of the chlorinated hydrocarbon.

40 The invention is illustrated by the following example but is not limited thereby. A mixture of C<sub>9</sub>–C<sub>14</sub> paraffins chlorinated to a chlorine content of 65% by weight and containing 1% by weight of epoxidised oil as heat stabiliser is stabilised according to the present invention by addition thereto of 0.25% of barium octyl phenol sulphide and 0.25% of pentaerythritol dioleate, the percentages being calculated on the weight of chlorinated paraffins. The stabilised chlorinated paraffin, when added in amount of 40% by weight to a mineral cutting oil provides a heavy duty cutting lubricant which gives no noticeable staining of ferrous metal parts.

45 50 55 60 65 70 75 80 85 90 95

What we claim is:

1. A stabilized lubricating oil additive which consists essentially of at least one liquid chlorinated paraffinic hy-

drocarbon containing 8-26 carbon atoms per molecule and about 25 to 70% by weight of chlorine, 0.1-5% of a metal alkyl phenate wherein said metal is selected from the group consisting of barium, calcium and magnesium, and 0.1-5% of an oil-soluble sequestering agent for heavy metals, the percentages of said phenate and said sequestering agent being calculated on the weight of said chlorinated paraffinic hydrocarbon.

2. A stabilized lubricating oil additive as claimed in claim 1 wherein said oil soluble heavy metal sequestering agent is selected from the group consisting of pentaerythritol esters of long chain fatty acids, alkyl phosphites and aryl phosphites.

3. A stabilized lubricating oil additive which consists essentially of at least one liquid chlorinated paraffinic hydrocarbon containing 8-26 carbon atoms per molecule and 40-70% by weight of chlorine, 0.1-1% of barium octyl phenol sulphide and 0.1-1% of pentaerythritol dioleate, the percentages being calculated on the weight of chlorinated paraffinic hydrocarbon.

4. A lubricating oil composition consisting essentially of a major amount of a mineral cutting oil and a stabilizing amount of a stabilized lubricating oil additive which consists essentially of at least one liquid chlorinated paraffinic hydrocarbon containing 8-26 carbon atoms per molecule and 40-70% by weight of chlorine, 0.1-1% of barium octyl phenol sulphide and 0.1-1% of pentaerythritol dioleate, the percentages being calculated on the weight of chlorinated paraffinic hydrocarbon.

5. The lubricating oil as claimed in claim 4 wherein

20 DANIEL E. WYMAN, *Primary Examiner.*

the stabilized lubricating oil additive comprises about 40% by weight of said lubricating oil.

6. A stabilised lubricating oil additive according to claim 1 wherein the said sequestering agent is a pentaerythritol ester of a long chain fatty acid.

7. A stabilised lubricating oil additive according to claim 1 wherein the said sequestering agent is a phosphite selected from the group consisting of alkyl phosphites and aryl phosphites.

10 8. A stabilised lubricating oil additive as claimed in claim 10 wherein the chlorinated paraffinic hydrocarbon component contains 40-70% by weight of chlorine.

9. A stabilised lubricating oil additive as claimed in claim 10 wherein the phenate is present to the extent of 0.1-1% by weight of the chlorinated paraffinic hydrocarbon.

15 10. A stabilised lubricating oil additive as claimed in claim 10 wherein the sequestering agent is present to the extent of 0.1-1% by weight of the chlorinated paraffinic hydrocarbons.

#### References Cited by the Examiner

##### UNITED STATES PATENTS

2,362,289 11/44 Mikeska ----- 252-42.7

##### FOREIGN PATENTS

487,630 10/52 Canada.

749,354 5/56 Great Britain.